

106-18.15

SR

XR 1,321,708

SEARCH ROOM

1,321,708.

P. R. BRADLEY.  
FIREPROOFING FOR AIRCRAFT.  
APPLICATION FILED MAR. 22, 1918.

Patented Nov. 11, 1919.

Fig.1



Fig.2.



Fig.3.



Fig.4.



Fig.5.



WITNESSES

Frederick Dichtl:  
Broadway.

INVENTOR

P.R. Bradley  
BY *M. M. Bradley*  
ATTORNEYS

1321708  
OR IN 428/249

Dec. 6 1919

## UNITED STATES PATENT OFFICE.

PARKER RICHARDSON BRADLEY, OF EAST ORANGE, NEW JERSEY, ASSIGNOR TO  
AIRCRAFT FIREPROOFING CORPORATION, OF NUTLEY, NEW JERSEY, A COR-  
PORATION OF DELAWARE.

## FIREPROOFING FOR AIRCRAFT.

1,321,708.

Specification of Letters Patent. Patented Nov. 11, 1919.

Application filed March 22, 1918. Serial No. 224,076.

*To all whom it may concern:*

Be it known that I, PARKER R. BRADLEY, a citizen of the United States, and a resident of East Orange, in the county of Essex and 5 State of New Jersey, have invented a new and Improved Fireproofing for Aircraft, of which the following is a full, clear, and exact description.

This invention relates to the fireproofing 10 of the cloth and wooden parts of flying machines by the application of a varnish-like liquid which imparts a fire-resisting surface thereto, the fireproofing coating being made of alginic acid products or an alginate as a 15 basis.

The general object of the invention is to provide a fireproof coating which is comparatively inexpensive, capable of being easily applied, and which has exceedingly 20 high fire-resisting qualities.

In carrying out the invention algin cellulose or the fiber-like product obtained as a by-product in the extraction of alginic acid may be ground into a fine powder and then 25 mixed with the alginic acid products or the alginates.

Preferably a layer of cellulose acetate dope in one or more coatings is applied to the cloth or wood surface of the aircraft, 30 and when dry a layer of one or more coatings of alginic acid or its alginates is applied, using preferably those which dry to a film insoluble in water. If desired, however, these layers may be reversed so that 35 the cellulose acetate dope will be on the outside and the coating of the alginic acid products or alginates will be directly on the cloth or wood surface. These alginic acid products may have their fire-resisting qualities increased by adding to them when in a 40 liquid state a suitable substance, such as boric acid or the salts generally used for fireproofing purposes, such as ammonium phosphate, sodium tungstate and the like.

Instead of using one or more first coatings 45 of cellulose acetate dope, good results can be obtained by using one or more coatings of cellulose nitrate dope and thereafter the alginic acid coatings are applied as described. The coatings of cellulose acetate or 50 cellulose nitrate may be omitted and the coatings of alginic acid products or alginates may be applied directly to the cloth sur-

faces of the aircraft, and the desired drum-like effects may be increased or diminished 55 by adding shellac or similar gum to the alginic acid products or the alginates, thereby effecting an enormous saving in the cost. Or another method consists in applying successive layers of cellulose nitrate dope and 60 cellulose acetate dope, the layers being applied in coatings successively after each dries, and then finally one or more layers of the fireproofing alginic acid products or 65 the alginates may be applied.

In the drawings, Figures 1 to 5 inclusive are fragmentary views showing the different methods of coating the part of an airship to be protected.

In the figures 1 is supposed to represent 70 a part of an airship that is to be fireproofed.

In Fig. 1 only a single layer 2 of several coatings is represented, which is a varnish-like liquid that hardens in a film form and 75 it is made from an alginic acid product or an alginate;

In Fig. 2 a double layer of protective material each of one or more coats is shown. The under layer 3 is cellulose acetate and 80 the outer layer is the same as the coating in Fig. 1. If desired the arrangements of the coatings 2 and 3 may be reversed, as shown in Fig. 4.

In Fig. 3 between the part 1 and the outer 85 layer 2 is a layer of cellulose nitrate 4.

In Fig. 4 the arrangement of the coatings 2 and 3, as shown in Fig. 2, is reversed.

In Fig. 5 the layers 5 and 6 are respectively coatings of cellulose nitrate and cellulose acetate and the outer layer 7 is composed of coatings of alginic acid products or alginates. 90

The foregoing are some of the various methods of protecting the surfaces of the 95 inflammable parts of an aircraft, but other combinations of layers may be employed, but an essential feature is the use of a fireproofing material embodying alginic acid.

Having thus described my invention, I 100 claim as new and desire to secure by Letters Patent:

1. The combination of a part to be fireproofed, with a surface layer thereon of a fireproofed material containing alginic acid 105 products.
2. The combination of a part of an air-

- craft to be fireproofed, with a plurality of layers of protective compound, one of the layers containing alginic acid products.
3. The combination of a part of an aircraft to be fireproofed, with a plurality of layers of protective compound, one of the layers containing alginic acid products, and another layer containing a cellulose compound.
4. The combination of a part of an aircraft to be fireproofed, with a fireproofing covering including a film forming varnish-like material containing an alginic acid product.
5. A protective material for the cloth or wooden parts of an aircraft, containing alginic acid products.
6. The combination of a part to be fireproofed, of a layer containing a cellulose compound and a second layer disposed over the first layer and containing alginic acid products.
7. The combination of a part to be fireproofed, of a plurality of layers of protective compound, one of the layers containing insoluble alginic acid products.

PARKER RICHARDSON BRADLEY,